# EUROPEAN PATENT SPECIFICATION

(11) **EP 2 471 977 B1**
(45) Date of publication and mention of the grant of the patent: **25.01.2017**
(21) Application number: 11195167.9
(22) Date of filing: 22.12.2011
(51) Int. Cl.: C25D 21/18, C23C 18/16, C23C 18/31

(54) **Method for removing impurities from plating solution**
Verfahren zum Entfernen von Verunreinigungen aus einer Metallisierungslösung
Procédé permettant de supprimer les impuretés d'une solution de placage

(30) Priority: 28.12.2010 JP 2010292150
(43) Date of publication of application: 04.07.2012
(73) Proprietor: Rohm and Haas Electronic Materials LLC, Marlborough, MA 01752 (US)
(72) Inventor: Hakiri, Yoshiyuki, Agano-shi, Niigata (JP)
(74) Representative: Hoggins, Mark Andrew

(56) References cited:
- DE-A1- 19 954 613
- JP-A- 2004 068 056
- INAI S ET AL: "Non-electrolytic tin-plating bath for formation of tin film on printed circuit board, contains organic sulfonic acid, thiourea, soluble stannous salt and hypophosphorous acid having preset molar ratio", WPI / THOMSON,, vol. 2004, no. 27, 4 March 2004 (2004-03-04), XP002637802,

## Description

### FIELD OF THE INVENTION

The present invention relates to a method for removing impurities from an electroless tin plating solution.

### BACKGROUND OF THE INVENTION

In recent years, an electroless tin plating is used broadly for mechanical components, flexible circuit boards and printed wiring boards, and for circuit patterns of electronic components. The electroless tin plating is often carried out as displacement tin plating on copper or copper alloys. While displacement tin plating is proceed, displaced copper becomes copper ion and dissolved in the plating solution, so that the copper ion is increased in the plating solutions during the progress of plating. Since such accumulating copper ions deteriorate the plating film and lowers the performance of the plating bath, so it is required to replacement the plating solution.

The conventionally known methods for control over plating solution are the batch method and the feed-and-bleed method. The batch method is a method to renew a plating bath when the plating bath is aged. Using the batch method, the plating bath must be renewed each time when the copper concentration increases and the bath performance decreases, so it causes various problems such as increasing the frequency of creating new plating baths, decreasing the productivity, and increasing the costs of descarding the aged solution. The feed-and-bleed method is a method of continuing plating while the plating solution overflows. Copper can be removed outside of the system via the overflow without stopping the plating operations, but large amounts of plating solution must be supplemented, which entails increase in costs.

Various techniques have been proposed as methods of resolving these problems. For example, JP05222540A discloses a method of precipitating a copper thiourea complex in the bath by cooling bath solution that has been partially removed. The copper thiourea complex is removed through filtration and the filtrate is returned to the original plating tank. JP2002317275A discloses a method whose operations are virtually identical with those in JP05222540A. In this method, the bath solution is cooled to a temperature below 40°C to precipitate copper thiourea complex. The copper thiourea complex is then filtered and removed.

JP10317154A discloses a method that uses a regeneration cell provided with an anode, a cathode andcation/anion exchange membrane, depositing copper on the anode in the electrolytic cell, adding tin ions passed through the cation exchange membrane into the plating solution after electroplated, then returing the solution to the plating tank. JP04276082A discloses a method of oxidation decomposition of copper thiourea complex.

However, the methods disclosed in JP0522540A and in JP2002317275A both require cooling steps, and a cooling facility for bath solution must be fitted to a conventional plating apparatus. The method disclosed in JP10317154A requires an electrolytic cell for regeneration, which complicates the apparatus. The method disclosed in JP04276082A requires chemicals and equipment for oxidation decomposition of the copper thiourea complex.

### PROBLEM SOLVED BY THE INVENTION

The objective of the present invention is to provide a method capable of efficiently removing impurities from a plating solution that has already been used in electroless tin plating without requiring separated equipment in order to remove impurities in a plating bath.

### MEANS OF SOLVING THE PROBLEM

The inventors conducted thorough research to resolve the above problems, and found that to add benzensulfonic acid, bensenesulfonic acid hydrate or salts threof into an electroless tin plating solution comprising thiourea or thiourea compounds, impurities in the plating bath could be removed efficiently from the bath without using specific equipment, and completed the present invention.

The present invention relates to a method for removing impurities from a tin plating solution comprising thiourea or thiourea compounds, wherein said solution has already been used in electroless tin plating and wherein said impurities are selected from copper, nickel, zinc, chromium, molybdenum and tungsten that have dissolved from the material to be plated, said method comprising: (i) adding benzenesulfonic acid, benzenesulfonic acid hydrate or salts thereof in the plating solution to generate a precipitate; and (ii) removing said precipitate from said solution.

In one embodiment, the solution has already been used in electroless plating on copper or copper-alloy.

In another embodiment, the precipitate is removed from the solution by circulating a part or all of the plating solution in a plating tank through a separation unit and filtrating by the separation unit a precipitate generated in the tank after adding benzenesulfonic acid, benzenesulfonic acid hydrate or salts thereof in the solution.

In another embodiment, the method is conducted in a multiple tank plating device comprising a main tank to plate the material, a precipitation tank to generate a precipitate, circulation pipes connected between the main tank and the precipitation tank so as to be capable of circulating electroless plating solution, and a solid-liquid separation unit placed between the precipitation tank and the main tank, wherein the method comprises the steps of; adding benzenesulfonic acid, benzenesulfonic acid hydrate or salts thereof to the plating solution in the precipitation tank, and separating a solid in the solution generated in the precipitation tank using the solid-liquid separation unit.

In another embodiment, the method is conducted in a single tank plating device comprising a plating tank to plate a material, circulation pipes connected to the plating tank so as to be capable of circulating a part or all of the plating solution, and a solid-liquid separation unit placed in the circulation route of the plating solution, wherein the method comprises the steps of; contacting the material to be plated with the plating solution in the plating tank, adding benzenesulfonic acid, benzenesulfonic acid hydrate or salts thereof to the plating solution in the plating tank, circulating the solution through the circulation pipes, and separating and removing a precipitate generated in the bath after adding benzenesulfonic acid, benzenesulfonic acid hydrate or salts thereof using the solid-liquid separation unit.

### EFFECTS OF THE INVENTION

Impurities in plating solution can be efficiently removed without requiring special equipment for cooling or oxidation decomposition through the use of the method pursuant to the present invention. Furthermore, plating solution can be used for a prolonged period of time since plating can be continuously carried out while removing impurities, and the frequency of discarding plating solution as well as the frequency of providing a fresh plating bath can be demonstrably reduced. As a result, the present invention can contribute to great enhancement of the industrial productivity.

### BRIEF DESCRIPTION OF THE DRAWINGS

Figure 1B is a result of SEM observation after the addition of benzenesulfonic acid (BSA)

### MODE OF IMPLEMENTING THE INVENTION

In the specification, °C represents degrees Centigrade, g represents gram, L represents liter, mL represents milliliter, dm represents decimeter, and µm represents micrometer. All amounts are in weight percentages unless otherwise specifically noted. "Plating solution" and "plating bath" in the specification have the same significance and are used interchangeably.

The target plating solution in the present invention is an electroless tin plating solution or an electroless tin alloy plating solution, in specifically, a plating solution that are capable of displacement tin plating or of displacement tin alloy plating on copper or on copper alloy. The electroless tin plating solution may contain a electroless tin plating solution further comprising other metals in addition to tin. The electroless tin plating solutions contain water soluble tin salts or water soluble tin salts and other metal salts as well as thiourea or thiourea compounds as complexing agents.

Any water soluble tin salts used in electroless tin plating solutions may be used in the plating solutions so long as they dissolve in water. Examples include stannous sulfate, stannous chloride, tin fluoroborate, tin alkanesulfonate, and tin alkanolsulfonate.

In addition, other metal salts such as salts of lead, copper, silver, bismuth and cobalt, may be used as additional metal salts that can be used with water soluble tin salts. Examples of the other metal salts include lead chloride, lead acetate, lead alkanesulfonate, copper chloride, silver nitrate, bismuth chloride, and cobalt sulfate.

The total amount of metal constituents in addition to tin and of tin in the plating solution would usually be in the range of 10 to 100 g/L as metal, preferably a range of 30 to 50 g/L.

Acid may be added to the electroless tin plating solution in order to dissolve tin and metal constituents other than tin. Acids that may be used in the plating solution include sulfuric acid, hydrochloric acid, alkanesulfonic acid, alkanolsulfonic acid, and aromatic sulfonic acid. These acids may be used alone or in combinations of two or more. The amount of acid that can be added to the plating solution would usually total in the range of 1 to 300 g/L, preferably a range of 50 to 100 g/L.

The electroless tin plating solution used in the present invention contains thiourea or thiourea compounds. These act as copper complexing agents. From the electrochemical perspective, these are well known to those skilled in the art as constituents that enable displacement tin plating on copper or copper alloys that are theoretically incapable of plating because of the standard electrode potential relationship. Thiourea that is readily available may be used, and commercial thiourea can be used as well.

Thiourea compounds are derivatives of thiourea. Examples include 1-methylthiourea, 1,3-dimethyl-2-thiourea, trimethylthiourea, diethylthiourea, N,N-diisopropyl thiourea, 1-(3-hydroxypropyl)-2-thiourea, 1-methyl-3-(3-hydroxypropyl)-2-thiourea, 1-methyl-3-(3-methoxypropyl)-2-thiourea, 1,3-bis (3-hydroxypropyl)-2-thiourea, allyl thiourea, 1-acetyl-2-thiourea, 1-phenyl-3-(2-thiazolyl)thiourea, benzyl isothiourea hydrochloride, 1-allyl-2-thiourea, and 1-benzoyl-2-thiourea. These thioureas or thiourea compounds may be used alone or in combinations of two or more. The amount of use of these thioureas or thiourea compounds would usually be in the range of 50 to 250 g/L, preferably a range of 100 to 200 g/L.

Electroless tin plating solution may contain antioxidants, surfactants and the like as required in addition to aforementioned constituents. Permissible examples of antioxidants that can be used include catechol, hydroquinone and hypophosphorous acid. Permissible examples of surfactants include one, two or more cationic, anionic, nonionic and amphoteric surfactants.

Displacement tin plating (electroless tin plating) is usually carried out by repairing the plating solution, setting the temperature to a range of 50 to 75°C, and immersing material to be plated with copper or copper alloy on the surface in plating solution for 120 to 300 seconds. The tin displaces the copper on the surface of material to be plated to form a tin film while the copper dissolves in the plating solution. Consequently, tin in the plating solution decreases as plating proceeds. Furthermore, the thiourea or thiourea compounds that are complexing agents are believed to form complexes with copper in the plating solution so that these thiourea or thiourea compounds also decrease as plating proceeds. Moreover, acid and other constituents decrease as the material to be plated is hoisted (pumped out), and they also decrease as plating proceeds. These constituents that decrease in the plating solution as plating proceeds are appropriately supplemented. However, copper increases as plating proceeds and its accumulation in the plating bath leads to deterioration of the plating film and a decline in the bath performance.

The present invention is characterized by the addition of benzenesulfonic acid, benzenesulfonic acid hydrate or salts thereof (hereinafter termed benzenesulfonic acid) to electroless tin plating solution in order to create a precipitate containing copper that inhibits the accumulation of copper in the plating solution. The concentration of copper ions in the plating solution can be reduced by adding benzenesulfonic acid to plating solution because copper ion complexes dissolve in the plating solution precipitate. The method pursuant to the present invention is far superior to conventional technology in that the temperature of the plating solution need not be lowered when creating a precipitate. While the specific reaction mechanism remains unclear, copper ions in the plating solution are believed to be found as complexes of thiourea or thiourea compounds, and the solubility of complexes of thiourea or thiourea compounds is lowered through the addition of benzenesulfonic acid, thereby resulting in the formation of precipitate without requiring a cooling operation.

Permissible examples of benzenesulfonic acid hydrates include benzenesulfonic acid 1-hydrate, benzenesulfonic acid 1.5-hydrate, and benzenesulfonic acid 2-hydrate. Arbitrary salts of benzenesulfonic acid and of benzenesulfonic acid hydrate are permissible. Concrete examples include sodium salts, potassium salts, and ammonium salts. Commercial benzenesulfonic acid may may also be used. Mixtures of benzenesulfonic acid, benzenesulfonic acid hydrate or salts thereof may also be used, and the amount used should be in the range of 5 to 200 g/L, preferably 20 to 100 g/L, more preferably 50 to 100 g/L. Precipitate does not form if the amount used is too low. An amount exceeding 20 g/L should be used in order to attain adequate precipitation. If the amount used is excessive, the tin precipitation state deteriorates and the bath performance is impaired, such as decline in the precipitation speed.

The method of the present invention is a method for removing impurities from a tin plating solution comprising thiourea or thiourea compounds, wherein adding benzenesulfonic acid, benzenesulfonic acid hydrate or salts thereof in the plating solution to generate a precipitate. The tin plating solution to which benzenesulfonic acid is added is a solution that has already been used in electroless tin plating. Either a plating solution in which electroless tin plating treatment has been completed or a solution whose electroless tin plating treatment is underway may be used. The impurities are copper or other metals (nickel, zinc, chromium, molybdenum, tungsten) that had dissolved from the material to be plated. The impurity would especially be copper, and copper can be effectively removed from plating solution. Insoluble constituents containing copper precipitate when benzenesulfonic acid is added to used plating solution in which the copper concentration has increased. Copper can be removed from the plating solution by removing such insoluble constituents. Arbitrary methods of removing insoluble constituents may be used, including filtration using a filter, precipitation separation, and centrifugal separation.

In one embodiment, the solution has already been used in electroless plating on copper or copper-alloy. As stated above, impurities, especially copper, can be removed from the plating solution through removal of precipitates by
adding benzenesulfonic acid. Plating solution can be reused following precipitate removal. Plating solution can be continuously used by supplementing other constituents that had been consumed or reduced in quantity. As a result, older plating solution need not be discarded, which contributes to enhanced industrial productivity.

In a further embodiment, the precipitate is removed from the solution by circulating a part or all of the plating solution in a plating tank through a separation unit and filtrating by the separation unit a precipitate generated in the tank after adding benzenesulfonic acid, benzenesulfonic acid hydrate or salts thereof in the solution. In this method, the circulation of electroless tin plating solution may be carried out while a plating film is formed as plating of material to be plated is continued, or it may be carried out as the plating operation is temporarily suspended. In addition, benzenesulfonic acid may be added while plating film is formed as plating of the material to be plated is continued, or it may be carried out as the plating operation is temporarily suspended. The addition of benzenesulfonic acid in the course of formation of plating film does not affect the characteristics of the plating film so long as the amount of plating solution in the plating tank is adequate. The fact that the plating operation need not be stopped during the addition of benzenesulfonic acid in the course of formation of a plating film as plating is continued or in the course of circulation of plating solution is desirable from the perspective of productivity. Any solid-liquid separation unit may be used so long as it is capable of separating precipitate that formed from plating solution. Filtration using a filter, precipitation separation, or centrifugal separation unit may be used. Here, the addition of benzenesulfonic acid to the plating solution that had deteriorated due to continuation of plating would preferably be carried out in the course of plating of material to be plated. The benzenesulfonic acid would preferably be added to plating solution in which metal ions such as copper, nickel, zinc, chromium, molybdenum or tungsten had dissolved from the material to be plated, resulting in a decline in the bath performance. As mentioned above, tin plating solution would be repaired and the formation of plating film would be carried out by adjusting the temperature of the plating solution to a temperature in the range of 50 to 75°C, followed by immersing the material to be plated that has copper or copper alloy on the surface in a plating solution for 120 to 300 seconds. Since copper ions dissolve in the plating solution as plating proceeds, the addition of benzenesulfonic acid, the circulation of plating solution and the capture removal of precipitate should be carried out at the necessary timing. Furthermore, constituents in the plating solution that had been consumed or diminished could be appropriately supplemented.

In a further embodiment, the method is conducted in a multiple tank plating device comprising a main tank to plate the material, a precipitation tank to generate a precipitate, circulation pipes connected between the main tank and the precipitation tank so as to be capable of circulating electroless plating solution, and a solid-liquid separation unit placed between the precipitation tank and the main tank, wherein the method comprises the steps of; (i) adding benzenesulfonic acid, benzenesulfonic acid hydrate or salts thereof to the plating solution in the precipitation tank, and (ii) separating a solid in the solution generated in the precipitation tank using the solid-liquid separation unit. This embodiment is characterized by the use of a multiple tank plating device furnished with a precipitation tank in order to form precipitates in addition to the main tank in which electroless plating is carried out. A minimum of two tanks are required, but three or more tanks may be used as needed. The main tank and the precipitation tank may be of arbitrary size and shape so long as they permit plating treatment and precipitate formation. The main tank and the precipitation tank are connected by piping to enable circulation of electroless plating solution between the two. The piping may be of arbitrary configuration so long as it permits circulation of plating solution. In addition, a solid-liquid separation unit may be placed between the precipitation tank and the main tank, and the precipitate that formed due to the addition of benzenesulfonic acid could then be separated. As indicated above, any arbitrary solid-liquid separation unit could be used.

Benzenesulfonic acid is added to plating solution in the precipitation tank in the first step. In the method of the present invention, benzenesulfonic acid may be added in the course of circulation of plating solution or benzenesulfonic acid may be added upon suspension of plating solution circulation. Furthermore, the plating operation in the main tank may be continued when adding benzenesulfonic acid, or the plating operation may be temporarily suspended. The addition of benzenesulfonic acid while continuing the plating operation is preferable from the perspective of productivity since plating need not be suspended. Furthermore, the temperature of the plating solution in the main tank should be in the range of 50 to 70°C, and the temperature of the plating solution in the precipitation tank may be the same temperature as that of the plating solution in the main tank or it preferably would be in a range 10°C above or below the liquid temperature in the main tank. Temperature control for regulating the temperature of the plating solution that had been returned to the main tank from the precipitation tank so as to regulate it to a temperature suitable for plating is facilitated by setting the temperature of the plating solution in the precipitation tank in this range. The method of capture of the precipitate that had been formed using the solid-liquid separation unit in the second step is as stated previously.

In a further embodiment, the method is conducted in a single tank plating device comprising a plating tank to plate a material, circulation pipes connected to the plating tank so as to be capable of circulating a part or all of the plating solution, and a solid-liquid separation unit placed in the circulation route of the plating solution, wherein the method comprises the steps of; (i) contacting the material to be plated with the plating solution in the plating tank, (ii) adding benzenesulfonic acid, benzenesulfonic acid hydrate or salts thereof to the plating solution in the plating tank, (iii) circulating the solution through the circulation pipes, and separating and removing a precipitate generated in the bath after adding benzenesulfonic acid, benzenesulfonic acid hydrate or salts thereof using the solid-liquid separation unit. This embodiment is characterized by the use of a single tank type of plating device for adding benzenesulfonic acid to a plating tank in which electroless plating is carried out to generate precipitate. The plating tank has a size and shape sufficient for plating treatment and for precipitate generation, but the use of a large-capacity tank would be preferable to the use of a multiple tank type of device when both operations are carried out concurrently. The circulation piping and the solid-liquid separation unit may have arbitrary configurations as mentioned above.

In the first step, the material to be plated is immersed in plating solution in a plating tank and displacement plating is carried out. The temperature of the plating solution in the plating tank should be in the range of 50 to 75°C. Copper ions that dissolved in the plating tank from the material to be plated accumulate as displacement plating proceeds in the plating tank. In the second step, benzenesulfonic acid is added to plating solution in the plating tank. When benzenesulfonic acid is added in the fifth method pursuant to the present invention, the plating operation may be continued in the plating tank or the plating operation may be temporarily suspended. The addition of benzenesulfonic acid while continuing the plating operation is preferable from the perspective of productivity since plating need not be suspended. In the third step, the precipitate generated in the plating tank is fed to the solid-liquid separation unit via the circulation piping where it is separated from the plating solution and removed. The circulation of plating solution must be conducted at least after the addition of benzenesulfonic acid. Furthermore, if aforementioned first to third steps are initiated in sequence, a subsequent step may be carried out without waiting for completion of the preceding step. For example, once material to be plated has been immersed in plating solution in the plating tank in the first step, benzenesulfonic acid addition, which constitutes the second step, may be carried out even while the immersion of material to be plated is continued.

### EXAMPLES

### Example 1

Electroless tin plating solution (basic bath 1) having the following composition was prepared.

### <Basic Bath 1>

Tin fluoroborate (as Sn²⁺) 30 g/L
Methanesulfonic acid 50 g/L
Hypophosphorous acid 15 g/L
Thiourea 100 g/L
Nonionic surfactant 30 g/L

A total of 15 g/L of copper powder was added to aforementioned tin plating solution, followed by heating for five hours at 65°C under stirring to complete a displacement reaction between copper and tin. The creation of electroless tin plating solution containing copper ions that had suffered deterioration was simulated. While aforementioned simulated electroless tin plating solution that had deteriorated was held at 65°C, 30 g/L of benzenesulfonic acid was added to the plating solution. Following the addition of benzenesulfonic acid, suspended material was generated in the plating solution. The suspended material precipitated while the plating solution was held at 65°C, and the supernatant that was then sampled was subjected to measurement of the copper concentration via atomic absorption analysis. The copper concentration that was measured was 9.5 g/L.

The same operations as in Example 1 were repeated except for the addition of 60 g/L of benzenesulfonic acid to aforementioned basic bath 1, after which the copper concentration was measured. The copper concentration was measured to be 6.6 g/L.

### Comparative Examples 1 to 5

The same operations as in Example 1 were repeated except for omitting benzenesulfonic acid addition to aforementioned basic bath 1 (Comparative Example 1) or adding 30 g/L of the compounds presented in Table 1 (Comparative Examples 2 to 5). Table 1 presents the results.

The copper concentration was measured only in Comparative Example 1 since no precipitate settled in any of Comparative Examples 1 to 5.

**TABLE 1**

| Example No. | Precipitant | Amount added (g/L) | Presence of precipitate | Copper concentration (g/L) |
|---|---|---|---|---|
| Example 1 | Benzenesulfonic acid | 30 | Present | 9.5 |
| Example 2 | Benzenesulfonic acid | 60 | Present | 6.6 |
| Comparative Example 1 | None | - | Absent | 14.7 |
| Comparative Example 2 | Paratoluene sulfonic acid | 30 | Absent | - |
| Comparative Example 3 | Naphthane sulfonic acid | 30 | Absent | - |
| Comparative Example 4 | Benzene carboxylic acid | 30 | Absent | - |
| Comparative Example 5 | Salicylic acid | 30 | Absent | - |

Aforementioned results indicate that the copper concentration in plating decreases as a result of the generation of precipitate upon the addition of benzenesulfonic acid.

### Examples 3, 4 and Comparative Example 6

Electroless tin plating solution having the following composition was prepared by modifying the composition of the plating bath from that in Example 1 (Basic Bath 2).

### <Basic Bath 2>

Tin methanesulfonate (as Sn²⁺) 30 g/L
Methanesulfonic acid 50 g/L
Hypophosphorous acid 15 g/L
Thiourea 100 g/L
Nonionic surfactant 30 g/L

The same operations as in Example 1 were repeated except for the addition to aforementioned basic bath 2 of benzenesulfonic acid in the quantities shown in Table 2, after which the copper concentration in the plating solution was measured. Table 2 shows the results.

**TABLE 2**

| Example No. | Precipitant | Amount added (g/L) | Presence of precipitate | Copper concentration (g/L) |
|---|---|---|---|---|
| Example 3 | Benzenesulfonic acid | 30 | Present | 10.6 |
| Example 4 | Benzenesulfonic acid | 60 | Present | 6.3 |
| Comparative Example 6 | None | - | Absent | 14.2 |

Aforementioned results indicate that the copper concentration in plating decreases as a result of the generation of precipitate upon the addition of benzenesulfonic acid even if the composition of the plating solution has been altered.

### Examples 5 and 6

Performance confirmation tests on plating solution were conducted following the removal of impurities through the addition of benzenesulfonic acid. Basic bath 1 used in Example 1 was prepared as the plating bath.

The preparation of an electroless tin plating solution containing copper ions that had undergone deterioration following completion of a displacement reaction of copper and tin through the addition of 7 g/L (Example 5) and 10 g/L (Example 6) of copper powder to basic bath 1, followed by heating for five hours, was simulated. Tin fluoroborate was added to aforementioned simulated, deteriorated, electroless tin plating solution in order to supplement the tin that had decreased due to displacement with copper, and the tin concentration was adjusted to 30 g/L. Displacement tin plating was carried out on material to be plated (TCP and COF in which pattern formation had been completed) for three minutes, fifteen seconds at 65°C using this plating solution, and SEM observation as well as film thickness measurement were completed. To aforementioned plating solution was added either 28 g/L (Example 5) or 40 g/L (Example 6) of benzenesulfonic acid, followed by adequate stirring, filtration, and removal of the precipitate that formed. Displacement plating was carried out using those baths following removal of the precipitate, SEM observation as well as film thickness measurement were completed, and the state was compared with that preceding the addition of benzenesulfonic acid (BSA). Table 3 presents the results. In addition, Figure 6 illustrates the SEM photographs before and after the addition of benzenesulfonic acid in Example 6. COF denotes "Chip on Film" while TCP denotes "Tape Carrier Package". Table 3 allows confirmation of decline in the copper concentration as well as improvement in the film thickness. Furthermore, improvement of the crystalline state was confirmed through Figure 1.

**TABLE 3**

| Example No. | Before BSA addition | | After BSA addition | |
|---|---|---|---|---|
| | Copper concentration (g/L) | Plating film thickness (µm) | Copper concentration (g/L) | Plating film thickness (µm) |
| Example 5 | 6.7 | 0.49 | 0.5 | 0.51 |
| Example 6 | 9.8 | 0.44 | 0.2 | 0.52 |

Recovery of the bath performance (recovery of the precipitation speed) through removal of copper using benzenesulfonic acid was confirmed in Examples 5 and 6.

## Claims

1. A method for removing impurities from a tin plating solution comprising thiourea or thiourea compounds, wherein said solution has already been used in electroless tin plating and wherein said impurities are selected from copper, nickel, zinc, chromium, molybdenum and tungsten that have dissolved from the material to be plated, said method comprising:
(i) adding benzenesulfonic acid, benzenesulfonic acid hydrate or salts thereof in the plating solution to generate a precipitate; and
(ii) removing said precipitate from said solution.

2. The method of claim 1 for removing copper impurities from a tin plating solution.

3. The method of claim 1, wherein said solution has already been used in electroless plating on copper or copper-alloy.

4. The method of claim 1, wherein said precipitate is removed from said solution by circulating a part or all of the plating solution in a plating tank through a separation unit and filtrating by the separation unit the precipitate generated in the tank after adding benzenesulfonic acid, benzenesulfonic acid hydrate or salts thereof in the solution.

5. The method of claim 1, conducted in a multiple tank plating device comprising a main tank to plate the material, a precipitation tank to generate a precipitate, circulation pipes connected between the main tank and the precipitation tank so as to be capable of circulating electroless plating solution, and a solid-liquid separation unit placed between the precipitation tank and the main tank, wherein the method comprises the steps of; adding benzenesulfonic acid, benzenesulfonic acid hydrate or salts thereof to the plating solution in the precipitation tank, and separating a solid in the solution generated in the precipitation tank using the solid-liquid separation unit.

6. The method of claim 1, conducted in a single tank plating device comprising a plating tank to plate a material, circulation pipes connected to the plating tank so as to be capable of circulating a part or all of the plating solution, and a solid-liquid separation unit placed in the circulation route of the plating solution, wherein the method comprises the steps of; contacting the material to be plated with the plating solution in the plating tank, adding benzenesulfonic acid, benzenesulfonic acid hydrate or salts thereof to the plating solution in the plating tank, circulating the solution through the circulation pipes, and separating and removing a precipitate generated in the bath after adding benzenesulfonic acid, benzenesulfonic acid hydrate or salts thereof using the solid-liquid separation unit.

7. The method according to any of the preceding claims, wherein benzenesulfonic acid, benzenesulfonic acid hydrate or salts thereof are added in a total amount of 5 to 200g/L.

8. The method according to claim 7, wherein benzenesulfonic acid, benzenesulfonic acid hydrate or salts thereof are added in a total amount of 20 to 100g/L.

9. The method according to claim 8, wherein benzenesulfonic acid, benzenesulfonic acid hydrate or salts thereof are added in a total amount of 50 to 100g/L.

## Patentansprüche

1. Ein Verfahren zum Entfernen von Verunreinigungen aus einer Zinnplattierungslösung, die Thioharnstoff oder Thioharnstoffverbindungen beinhaltet, wobei die Lösung bereits in stromloser Zinnplattierung verwendet wurde und wobei die Verunreinigungen aus Kupfer, Nickel, Zink, Chrom, Molybdän und Wolfram ausgewählt sind, welche aus dem zu plattierenden Material herausgelöst wurden, wobei das Verfahren Folgendes beinhaltet:
(i) Zugeben von Benzolsulfonsäure, Benzolsulfonsäurehydrat oder Salzen davon in die Plattierungslösung zum Erzeugen eines Präzipitats; und
(ii) Entfernen des Präzipitats aus der Lösung.

2. Verfahren gemäß Anspruch 1 zum Entfernen von Kupferverunreinigungen aus einer Zinnplattierungslösung.

3. Verfahren gemäß Anspruch 1, wobei die Lösung bereits in stromloser Plattierung auf Kupfer oder Kupferlegierung verwendet wurde.

4. Verfahren gemäß Anspruch 1, wobei das Präzipitat aus der Lösung entfernt wird, indem ein Teil der Plattierungslösung oder die ganze Plattierungslösung in einem Plattierungstank durch eine Trenneinheit zirkulieren gelassen wird und das in dem Tank nach dem Zugeben von Benzolsulfonsäure, Benzolsulfonsäurehydrat oder Salzen davon in die Lösung erzeugte Präzipitat durch die Trenneinheit filtriert wird.

5. Verfahren gemäß Anspruch 1, durchgeführt in einer Plattierungsvorrichtung mit mehreren Tanks, die einen Haupttank zum Plattieren des Materials, einen Präzipitierungstank zum Erzeugen eines Präzipitats, Zirkulationsrohre, die den Haupttank und den Präzipitierungstank verbinden, um eine Lösung für stromlose Plattierung zirkulieren lassen zu können, und eine Fest-Flüssig-Trenneinheit, die zwischen dem Präzipitierungstank und dem Haupttank platziert ist, beinhaltet, wobei das Verfahren die Schritte des Zugebens von Benzolsulfonsäure, Benzolsulfonsäurehydrat oder Salzen davon zu der Plattierungslösung in dem Präzipitierungstank und das Trennen eines in dem Präzipitierungstank erzeugten Feststoffs in der Lösung unter Verwendung der Fest-Flüssig-Trenneinheit beinhaltet.

6. Verfahren gemäß Anspruch 1, durchgeführt in einer Ein-Tank-Plattierungsvorrichtung, die einen Plattierungstank zum Plattieren eines Materials, Zirkulationsrohre, die mit dem Plattierungstank verbunden sind, um einen Teil der Plattierungslösung oder die ganze Plattierungslösung zirkulieren lassen zu können, und eine Fest-Flüssig-Trenneinheit, die in der Zirkulationsroute der Plattierungslösung platziert ist, beinhaltet, wobei das Verfahren die Schritte des In-Kontakt-Bringens des zu plattierenden Materials mit der Plattierungslösung in dem Plattierungstank, das Zugeben von Benzolsulfonsäure, Benzolsulfonsäurehydrat oder Salzen davor zu der Plattierungslösung in dem Plattierungstank, das Zirkulierenlassen der Lösung durch die Zirkulationsrohre und das Trennen und Entfernen eines in dem Bad nach dem Zugeben von Benzolsulfonsäure, Benzolsulfonsäurehydrat oder Salzen davon erzeugten Präzipitats unter Verwendung der Fest-Flüssig-Trenneinheit beinhaltet.

7. Verfahren gemäß einem der vorhergehenden Ansprüche, wobei Benzolsulfonsäure, Benzolsulfonsäurehydrat oder Salze davon in einer Gesamtmenge von 5 bis 200 g/l zugegeben werden.

8. Verfahren gemäß Anspruch 7, wobei Benzolsulfonsäure, Benzolsulfonsäurehydrat oder Salze davon in einer Gesamtmenge von 20 bis 100 g/l zugegeben werden.

9. Verfahren gemäß Anspruch 8, wobei Benzolsulfonsäure, Benzolsulfonsäurehydrat oder Salze davon in einer Gesamtmenge von 50 bis 100 g/l zugegeben werden.

## Revendications

1. Une méthode destinée à éliminer des impuretés d'une solution de placage d'étain comprenant de la thiourée ou des composés de thiourée, où ladite solution a déjà été utilisée pour un placage d'étain non électrolytique et où lesdites impuretés sont sélectionnées parmi du cuivre, du nickel, du zinc, du chrome, du molybdène et du tungstène s'étant dissous depuis le matériau à plaquer, ladite méthode comprenant le fait :
(i) d'ajouter de l'acide benzènesulfonique, de l'acide benzènesulfonique hydraté ou des sels de ceux-ci dans la solution de placage afin de générer un précipité ; et
(ii) d'éliminer ledit précipité de ladite solution.

2. La méthode de la revendication 1 destinée à éliminer des impuretés de cuivre d'une solution de placage d'étain.

3. La méthode de la revendication 1, où ladite solution a déjà été utilisée pour un placage non électrolytique sur du cuivre ou un alliage-cuivre.

4. La méthode de la revendication 1, où ledit précipité est éliminé de ladite solution en faisant circuler une partie ou l'ensemble de la solution de placage dans une cuve de placage via une unité de séparation et en filtrant grâce à l'unité de séparation le précipité généré dans la cuve après l'ajout de l'acide benzènesulfonique, de l'acide benzènesulfonique hydraté ou des sels de ceux-ci dans la solution.

5. La méthode de la revendication 1, mise en oeuvre dans un dispositif de placage à cuves multiples comprenant une cuve principale pour plaquer le matériau, une cuve de précipitation pour générer un précipité, des conduits de circulation raccordés entre la cuve principale et la cuve de précipitation de façon à être en mesure de faire circuler une solution de placage non électrolytique, et une unité de séparation solide-liquide placée entre la cuve de précipitation et la cuve principale, où la méthode comprend les étapes consistant : à ajouter de l'acide benzènesulfonique, de l'acide benzènesulfonique hydraté ou des sels de ceux-ci à la solution de placage dans la cuve de précipitation, et à séparer un solide dans la solution généré dans la cuve de précipitation à l'aide de l'unité de séparation solide-liquide.

6. La méthode de la revendication 1, mise en oeuvre dans un dispositif de placage à cuve unique comprenant une cuve de placage pour plaquer un matériau, des conduits de circulation raccordés à la cuve de placage de façon à être en mesure de faire circuler une partie ou l'ensemble de la solution de placage, et une unité de séparation solide-liquide placée sur la trajectoire de circulation de la solution de placage, où la méthode comprend les étapes consistant : à mettre le matériau à plaquer en contact avec la solution de placage dans la cuve de placage, à ajouter de l'acide benzènesulfonique, de l'acide benzènesulfonique hydraté ou des sels de ceux-ci à la solution de placage dans la cuve de placage, à faire circuler la solution via les conduits de circulation, et à séparer et éliminer un précipité généré dans le bain après l'ajout de l'acide benzènesulfonique, de l'acide benzènesulfonique hydraté ou des sels de ceux-ci à l'aide de l'unité de séparation solide-liquide.

7. La méthode selon n'importe lesquelles des revendications précédentes, où l'acide benzènesulfonique, l'acide benzènesulfonique hydraté ou des sels de ceux-ci sont ajoutés dans une quantité totale de 5 à 200 g/L.

8. La méthode selon la revendication 7, où l'acide benzènesulfonique, l'acide benzènesulfonique hydraté ou des sels de ceux-ci sont ajoutés dans une quantité totale de 20 à 100 g/L.

9. La méthode selon la revendication 8, où l'acide benzènesulfonique, l'acide benzènesulfonique hydraté ou des sels de ceux-ci sont ajoutés dans une quantité totale de 50 à 100 g/L.
